

Feb. 10, 1931.

M. J. DE FRANCE

1,792,362

RUBBER BALL

Filed Feb. 29, 1928

Fig. I.



Fig. II.



Fig. III.



Fig. IV.



WITNESS

A.B. Wallace.

INVENTOR

Murrell J. De France  
by Christy and Christy  
his attorneys

## UNITED STATES PATENT OFFICE

MURRELL J. DE FRANCE, OF JEANNETTE, PENNSYLVANIA, ASSIGNOR TO PENNSYLVANIA RUBBER COMPANY, OF JEANNETTE, PENNSYLVANIA, A CORPORATION OF PENNSYLVANIA

RUBBER BALL

Application filed February 29, 1928. Serial No. 257,932.

My invention relates to improvements in the method of making inflated rubber shells and specifically rubber playing balls. I employ the term rubber in its popular and non-technical sense. "Rubber balls" in the common meaning of the term are hollow and ordinarily thin-walled spheres of a composition which includes caoutchouc and certain mineral substances, into which composition a quantity of sulphur is introduced. The ball when shaped is vulcanized, and the wall of the finished ball has qualities of softness, elasticity, and durability, to the attainment of which the composition of materials and the dimensions and proportions of the ball have been carefully worked out. While not limited in its application to rubber playing balls of any particular sort, my invention finds practical application in the making of tennis balls, and in such particular application I shall show and describe it.

In the accompanying drawings Fig. I is a view in central section of one of the two hemispherical shells which go to make up a tennis ball. It may be understood that the shell as it is here shown is a shell of semi-cured rubber, as it comes from the mold. Fig. II is a diagrammatic view in vertical section, illustrating a convenient method of coating the shell of semi-cured rubber interiorly with gelatin. Fig. III is a view corresponding to Fig. I and showing the shell after it has been coated successively with gelatin and with rubber. Fig. IV is a fragmentary view in section, illustrating the union of the edges of companion hemispherical shells, to form the ball. The figures, all of them are diagrammatic, in that the coatings are shown as of exaggerated thickness.

A tennis ball is, it will be understood, a thoroughly standardized article. It is a hollow, thin-walled, rubber ball, inflated, and covered externally with felt. Its dimensions, its wall thickness, its degree of inflation, its weight, and the characteristics which adapt it to its intended use, are most minutely defined. Problems arise, to produce economically the standard article, and to give durability in largest measure to the ball which initially comes up to the standard.

A thin wall of rubber such as that of a tennis ball is by no means impervious to gas, particularly when, as is the case with a tennis ball, the pneumatic pressures upon its opposite surfaces are unequal. And because the rubber wall is permeable, it has long since been the practice, in order to prolong the life of the tennis ball, to coat the wall interiorly with a preparation of gelatin. Such an inner coating, without undue prejudice to the quality and character of the ball in other respects, renders it tighter to resist the escape of gas. And, since the ball is inflated; that is to say, since it contains gas under super-atmospheric pressure, the life of the ball is by this expedient prolonged.

In the making of tennis balls, it is the universal practice to shape hemispherical shells of green rubber and, after partial and incomplete vulcanization, to unite two shells edge to edge, and to complete vulcanization after the ball itself has so been completely shaped. And in making balls with interior coatings of gelatin, it is the universal practice to apply the gelatin to the hemispherical and incompletely cured shells. The gelatin is ordinarily prepared in the form of an aqueous solution, and it may then be applied in various ways, as by painting or spraying the solution upon the surface of the rubber, or by dipping the rubber article in a bath of gelatin solution. The hemispherical shell of semi-cured rubber, as it comes from the mold, is shown in Fig. I of the drawings. My preferred way of applying gelatin to the rubber shell, is illustrated in Fig. II. A reservoir 4 is provided, adapted to contain a suitable quantity of gelatin solution. The reservoir is jacketed, so that hot water may circulate around the body of gelatin solution within the reservoir. From the bottom of the reservoir a valved and open-ended tube 5 extends downward. The reservoir otherwise closed, is provided through its top with two valve-controlled connections 6 and 7, one to a source of air under pressure, the other to pressure-reducing means. In operation the semi-cured shell 1 is placed beneath the reservoir, its rim carefully leveled, and tube 5 at its lower end closely adjacent to the mid-point of the con-

cavity of the shell. The valves in tubes 5 and 6 then are opened, whereupon hot gelatin solution flows through the tube and fills the shell. When the flood of gelatin solution rising within the shell reaches the edge, the valve in tube 6 is closed and the valve in tube 7 is opened. Thereupon the flood of gelatin is drawn back from the shell into the cylinder 4 again, leaving however a thin film, coating the shell interiorly. It is of great importance that the very edge 12 be not coated with gelatin, and by employing the apparatus which I have described the coating may be done expeditiously and with precision, and the edge 15 12 be left uncoated.

The strength of the solution of gelatin and its temperature are so far under control as to afford a liquid of the proper degree of viscosity and a coating of desired thickness.

Because the gelatin is applied in a condition of solution, it is necessary to interpose in the course of ball manufacture, a step of drying; and, since an aqueous solution of gelatin is very slow to dry, a very serious 20 delay is so injected into the progress of the operation of ball making. My invention includes a subjecting of the shell when coated with gelatin solution to ultra-violet rays emanating from a suitable light source. I have discovered that, according to what principle I know not, ultra-violet rays have the remarkable effect of causing the gelatin coating spread upon the rubber to dry in a relatively brief interval of time. In consequence, 25 the procedure of making tennis balls is very considerably hastened and that with economy in production as a whole.

The solution which I preferably employ for coating the inner surface of the ball contains in addition to gelatin a substance which is a coagulant of gelatin, acting upon the gelatin with an effect akin to tanning. Various substances possess this property or quality, typical among which is formaldehyde. If 30 formaldehyde be present in the solution, not only will the coating dry, but it will become tough and leathery to a degree which the gelatin alone never would attain, and, being so modified in its character and quality, it is even more serviceable to the intended end. I have found that if one or another of certain substances be used as the coagulant, the effect of the ultra-violet rays acting in the manner described will be more immediate and more pronounced, and among the substances which I have so found to be effective, I enumerate the following: formaldehyde, potassium dichromate, sodium dichromate, alcohol, potassium iodide, ferrous sulphate, and 35 tannic acid. I do not consider this to be an exhaustive catalogue, but merely indicative of substances which have the effect described.

According to my preferred mode of procedure, I shape the hollow hemispheres of 40 rubber and semi-cure them in usual manner,

70 coat them interiorly with gelatin solution, and deposit them on a travelling support. This support may conveniently be an endless belt, and I cause it as it travels to bear the hemispheres directly beneath a dome-like reflector, within which is arranged a light source which emanates ultra-violet rays. Passing at moderate rate beneath the influence of such a light source so situated, the hemispheres pass on with their gelatin coatings in effectively dried condition.

75 Various expedients are resorted to for effecting proper inflation of the tennis ball. One expedient is to enclose within the ball when the component hemispherical shells are brought together, chemical substances which reacting shall generate gas, and, the quantities being accurately measured, the quantity of gas so generated is predetermined, and it is sufficient both to give the desired tension from within while the ball is undergoing its ultimate vulcanization, and also to afford for the finished ball the desired degree of inflation. Specifically, in the procedure in which I have developed this invention, separate pellets of predetermined content one of sodium nitrite and the other of ammonium chloride, are closed within the ball and with them a small and measured quantity of water. Reaction occurs under the 80 heat of the vulcanizing operation, nitrogen is generated, and the desired effect is gained.

85 In following such procedure, if the hemispheres be interiorly faced with gelatin, the inflation creating materials so introduced will have a localized deteriorating effect upon the gelatinous coating, and this will tend to impair the quality of the finished ball.

90 My further invention lies in adding to the interiorly coated hemisphere one interior coating more, a coating protective of the gelatin against deterioration by introduced inflation-creating materials, and preferably this second coating is a coating of rubber. The rubber is preferably applied in fluid condition, and this is attained by dissolving it in a suitable solvent, benzene, for example.

95 I conveniently spray the rubber solution upon the gelatin-coated inner surface of the hemisphere, by bringing the hemisphere to place above a nozzle and projecting the solution in a spray from the nozzle. The solvent quickly evaporates and the rubber coating remains, of controlled thickness, effecting no impairment of the article for its intended purpose, and rendering the hemispherical shell better adapted for the further steps of manufacture.

100 Incidentally, I preferably so coat, not the interior surface only of the hemisphere, but the edge 12 as well, so that when two hemispheres are brought together their edges are faced with green rubber—"rubber cement", it is termed,—and in consequence an im- 105

proved weld or union of the edges is effected.

The rubber in solution may have sulphur mingled with it, so that it too is susceptible to vulcanization, but it will not itself ordinarily have undergone any appreciable vulcanization, although inevitably, in theory at least, such a change must be in progress, wherever rubber and sulphur have been brought into association.

10 The ball which emerges from the vulcanizing mold will be a hollow ball whose exterior and interior surfaces are of rubber and which contains within its structure a layer of substance impenetrable by gas, namely a layer of 15 gelatin, preferably indurated by the special treatment described. In tennis ball manufacture, this product of the vulcanizing mold will be covered in usual manner with felt.

Fig. I of the drawings shows the molded 20 and semi-cured hemispherical shell of rubber. Fig. II illustrates the step of coating with gelatin. Fig. III shows the hemispherical shell coated interiorly with rubber. The shell itself is indicated at 1, and from it, as 25 will be perceived, the flash or fin 11, incident to the initial molding operation, has been trimmed away. The coating of gelatin is indicated at 2, and the inner coating of rubber is indicated at 3. It will be observed that 30 this inner coating of rubber faces not only the interior hemispherical surface, but at 33 it faces the edges of the shells as well. Fig. IV illustrates the meeting of the two hemispherical shells edge to edge, and it will 35 be seen that the meeting of the two edge coatings 33 of the two shells facilitates and assures the integration of the shells to form the complete ball when the assembled blank is brought within the mold and vulcanized. 40 During vulcanization the gas generated within the hollow attains a pressure adequate to vulcanization, and when the finished ball returns to atmospheric temperature the contained pressure is adequate to the ends in 45 view.

I claim as my invention:

1. As a step in the manufacture of an inflated rubber article the method herein described, which consists in spreading upon a 50 wall of rubber a coating of a solution of gelatin, drying the applied coating under ultraviolet rays, and applying over the dried coating a second coating of rubber.
2. In the manufacture of an inflated rubber article the method herein described, which consists in forming a hollow blank of incompletely vulcanized rubber, coated interiorly with successive layers of gelatin and of rubber, inclosing within the blank water and 60 chemically reactive gas generative substances, and subjecting the blank within a mold to vulcanizing temperature.
3. In the manufacture of a tennis ball the method herein described which consists in 65 forming two hemispherical shells of incom-

pletely vulcanized rubber, coating the shells interiorly with gelatin, coating the shells over the gelatin coating and over their edges as well with rubber cement, bringing the two shells together edge to edge within a mold and with quantities of gas-generating substance and of water in the interior space, and raising the mold enclosed article to vulcanizing temperature.

In testimony whereof I have hereunto set 70 my hand.

MURRELL J. DE FRANCE.

80

85

90

95

100

105

110

115

120

125

130